

## [54] METHOD OF MAKING HOLLOW CAST ARTICLES FROM METAL ALLOYS HAVING LONG FREEZING RANGES

[75] Inventors: Richard H. Krock, Weston; William J. Richmond, Reading, both of Mass.

[73] Assignee: P. R. Mallory &amp; Co. Inc., Indianapolis, Ind.

[22] Filed: Jan. 11, 1972

[21] Appl. No.: 217,014

[52] U.S. Cl. .... 29/526.5, 29/527.5, 29/527.6, 164/125, 249/197

[51] Int. Cl. .... B22d 27/04

[58] Field of Search: 164/69, 126; 29/526.4, 29/526.5, 527.5, 527.6; 249/197

## [56] References Cited

## UNITED STATES PATENTS

3,548,915 12/1970 Richmond et al. .... 164/68

1,607,475 11/1926 Otto ..... 29/526.4 UX  
3,557,437 1/1971 St. Clair ..... 164/69 X

Primary Examiner—Charles W. Lanham

Assistant Examiner—D. C. Reiley, III

Attorney, Agent, or Firm—Richard H. Childress; Charles W. Hoffmann; Robert F. Meyer

## [57] ABSTRACT

A technique for improving the physical properties of thin walled castings and reduction or avoidance of hot tearing in such castings involves casting in the inverted position, preferably using no core. The exterior of the casting is contoured to the shape of a metal mold which causes rapid solidification with resultant improved soundness and improved physical properties. Metal is then removed from the interior of the casting for example by machining to form the desired wall thickness.

6 Claims, 4 Drawing Figures



PATENTED MAY 7 1974

3,808,671



FIG. 1



ALUMINUM-BERYLLIUM PHASE DIAGRAM



FIG. 4

## METHOD OF MAKING HOLLOW CAST ARTICLES FROM METAL ALLOYS HAVING LONG FREEZING RANGES

The invention described herein was made in the course of, or under, a subcontract issued under Prime Contract W-7405-ENG-48 with the United States Energy Commission.

### SUMMARY OF THE INVENTION

The following method is used to improve the physical properties of relatively thin walled hollow castings and prevent hot tearing caused by cores in alloys having long freezing ranges. The casting is inverted from the normal casting position and preferably no core is used. The exterior of the casting is contoured to the shape of a metal mold which causes rapid solidification with resultant improved soundness and high physical properties. The center section acts as a riser to feed the outer shell and minimize interdendritic shrinkage and hot tearing. The interior is then machined out to form the desired wall thickness.

### DRAWINGS

FIG. 1 is a view of a mold set up for the casting of hollow sections according to the prior art.

FIG. 2 is a sectional view of the coreless casting method according to the present invention.

FIG. 3 is a view of a casting produced in accordance with the present invention.

FIG. 4 is a view of the beryllium-aluminum phase diagram illustrating the long freezing of this system.

### BACKGROUND OF THE INVENTION

In accordance with techniques of the prior art, alloys having long freezing ranges have been difficult to cast in thin section sizes in hollow configurations. The problems involved include hot tearing of the metal during casting. Also the resulting castings often contain shrinkage resulting from the difference in dimensions between the material when first cast as compared to the room temperature dimensions.

The common method of casting hollow members with alloys having long freezing ranges is shown in FIG. 1. A metal mold 10 made for example, of copper, steel or graphite includes a base portion 11, a cylindrical portion 12, and a core 15 is utilized to form the casting. If desired an insulating sleeve 17 for example, made of alumina or zirconia also can be used to define a hot top portion 18. Alternatively the hot top portion may be defined by the interior surface 13 of material 12. Water cooling systems (not shown) are sometimes utilized in connection with the prior art construction of FIG. 1.

However, with or without water cooling, hot tearing has always been a problem in casting according to the prior art construction with alloys having a long freezing range. Additionally, interdendritic shrinkage and shrinkage resulting from the dimensional differences between the as cast material and the material at lower room temperature are serious problems.

In accordance with the present invention it has been found that if the casting is inverted from the position shown in FIG. 1 and the core is not used the problems of shrinkage and hot tearing are eliminated or are substantially reduced.

As shown in FIG. 2, a mold 100 may be used having a base portion 101 and a cylindrical portion 102. Base

portion 101 defines the external surface of the casting at 103. The preferred mold material or the mold 100 is metal and most preferably it is made of steel, copper, or cast iron. Graphite may also be used if desired.

A hot top section 120 is provided in conjunction with portion 102. If desired an insulating sleeve 121 may be provided which may be made of for example alumina or zirconia.

While not being wished to be bound by any particular theory, it is believed that the improvements observed according to the casting technique of the present invention are achieved because the massive mold section 101 removes heat very rapidly as a result of which rapid solidification occurs at and near the surface 103. The center section 134 of casting 130 acts as a riser to feed the outer shell 131. As a result interdendritic shrinkage and hot tearing are minimized, and good physical properties are obtained at and near the surface of the casting, particularly for wall thickness less than about one-half inch.

After the casting operation the casting 130 is removed from the mold and is machined to desired dimensions. If desired the casting may be simply cropped off along the line 132 of FIG. 3, and then the leg portion 131 machined as illustrated, removing center section 134. Alternatively it may be desirable for the leg portion 131 to be longer including portion 135 in which case the casting will not be cropped at 132 and the machining will include the portion 137, as illustrated.

Obviously the particular casting configurations shown are by way of example, only, and a wide variety of configurations may be cast and machined to desired shape according to the present invention.

The present invention is applicable to a wide variety of alloys having a long freezing range, generally having a freezing range of at least about 500° C and preferably above 550° C. Examples include the beryllium-aluminum system shown in FIG. 4, including alloying additives such as copper, magnesium, silicon, precious metals, either singly or in combination, preferably not totaling above about 10 percent, which may be used for various purposes such as strengthening the aluminum matrix and facilitating nucleation during casting. The preferred alloys contain about 80 to about 95 atomic percent beryllium.

Additional alloying systems include aluminum-germanium preferably about 90 to 99 atomic percent germanium, gold-germanium preferably 85 to 99 atomic percent germanium, lead-germanium preferably 75 to 99 atomic percent germanium, gallium-germanium preferably 20 to 99 atomic percent germanium, silver-silicon preferably 65 to 99 atomic percent silicon and silicon-tin preferably 10 to 99 atomic percent silicon.

Insofar as preparing the molten metal for casting is concerned, a wide variety of techniques are available for this purpose. For beryllium-aluminum alloys, one method which is particularly advantageous is disclosed in U.S. Pat. No. 3,548,915 which is hereby incorporated into the present application by reference as one exemplary method of preparing the alloys for casting.

As an example of the present invention, a beryllium-aluminum alloy containing 75 weight percent beryllium about 24.7 weight percent aluminum alloy and about 0.3 percent platinum was heated to a melting temperature of about 1,400° C and was then poured into the

mold shown in FIG. 2 at about 1,200° C. A similar composition was poured into the mold shown in FIG. 1 having been heated to the same melting and pouring temperatures, and otherwise similarly processed.

The resulting mechanical properties for the alloy cast in the mold shown in FIG. 1 was 19,000 psi ultimate tensile strength; 0.2 percent yield strength, 18,000 psi from a tensile bar taken near the surface of core 15. Radiography revealed extreme shrinkage and porosity adjacent the core in the resulting casting.

The castings produced according to the design in FIG. 2 had a tensile strength of 32,000 psi and 25,000 psi 0.2 percent yield strength from a tensile bar taken from section 131. Radiography revealed very little shrinkage and porosity in the channel portion formed adjacent surface 103 in the lower portion of the mold 101.

What is claimed is:

1. A method of making a relatively thin walled hollow tapered cast article from molten metal having an extremely long freezing range, the method comprising the steps of feeding molten metal having a freezing range of about 500° C or longer into a mold having an inverted tapered mold cavity and having a massive tapered bottom portion capable of withdrawing heat more rapidly from molten metal than an adjacent insu-

lated upper portion of the mold, solidifying molten metal in the massive bottom portion of the mold where heat is more rapidly withdrawn from the molten metal than withdrawn in the adjacent insulated portion of the mold and wherein molten metal at about the center of the mold acts as riser means and then solidifying the remainder of the molten metal in the mold to form a solidified casting of solid taper cross-section containing a minimum of hot tearing, removing the solidified casting from the mold, and removing solidified metal from the interior of the solidified casting to form the hollow cast article.

2. The method of claim 1, wherein the molten material having a freezing range of about 500° C or longer is a molten alloy selected from the group consisting of Be base alloys, Si base alloys or Ge base alloys.

3. The method of claim 2, wherein the molten alloy is a Be base alloy containing A1.

4. The method of claim 1, wherein the molten material is poured into the mold.

5. The method of claim 1, wherein the mold is a coreless mold.

6. The method of claim 5, wherein the solidified casting of the alloy experiences a minimum of interdendritic shrinkage.

\* \* \* \* \*

30

35

40

45

50

55

60

65

UNITED STATES PATENT OFFICE  
CERTIFICATE OF CORRECTION

Patent No. 3808671 Dated May 7, 1974

Inventor(s) Richard H. Krock & William J. Richmond

It is certified that error appears in the above-identified patent and that said Letters Patent are hereby corrected as shown below:

Col. 1, line 7, after "States" insert ---Atomic---.

Col. 1, line 32, after "freezing" insert ---range---.

Col. 2, line 13, change "rapdily" to ---rapidly---.

Col. 4, line 4, after "than" insert ---is---.

Signed and sealed this 10th day of September 1974.

(SEAL)

Attest:

MC COY M. GIBSON, JR.  
Attesting Officer

C. MARSHALL DANN  
Commissioner of Patents